

## UNITED STATES PATENT OFFICE

1,992,655

## ALLOY

Edward F. Fischer, Cleveland, Ohio, assignor, by  
mesne assignments, to Magnesium Develop-  
ment Corporation, a corporation of Delaware

No Drawing. Application February 6, 1934,  
Serial No. 709,970

4 Claims. (Cl. 75—1)

This invention relates to magnesium base alloys and it is particularly concerned with those alloys containing antimony.

Magnesium as a structural material is known chiefly for its extreme lightness of weight, the specific gravity of the pure metal being about 1.75. The metal, however, does not cast well and considerable difficulty is encountered in working it as compared to aluminum, for example. A further objection is the comparatively low strength of the metal, the tensile strength in the as cast condition being about 13,000 pounds per square inch while the rolled metal only has a tensile strength of about 25,000 pounds per square inch. Such limitations in strength have restricted the wider use of the metal.

It is an object of my invention to utilize the inherently advantageous properties of the pure metal and at the same time to overcome some of the handicaps. A particular object is to improve the strength of the metal without substantially diminishing its ductility.

I have found that from about 0.5 to 5 per cent of antimony can be added to magnesium thereby causing a surprisingly large increase in strength. The weight of the alloy does not differ substantially from that of the unalloyed metal.

For many purposes an extruded product is desirable either by reason of low production cost or because the intricate shape of the article renders difficult other methods of working. I have found that the magnesium-antimony alloys herein described may be readily extruded under the same conditions employed in handling the pure metal while at the same time a material is obtained which has appreciably higher strength

values than the pure magnesium. A magnesium-antimony alloy, for example, containing about 1 per cent of antimony had a tensile strength of about 33,600 pounds per square inch and an elongation of about 3.5 per cent in two inches in the as-extruded condition. An increase in the antimony content of 4 per cent served to further increase the strength, a value of about 36,400 pounds per square inch being obtained. The elongation in this case was 5 per cent, somewhat more than in the alloy of lower antimony content. For most purposes I prefer to use between about 1 and 4 per cent of antimony.

The alloy may be prepared in any manner known to those skilled in the art but preferably I use a "rich alloy" for the purpose of adding the antimony because of the vigorous action between molten magnesium and metallic antimony. The use of a "rich" alloy obviates this difficulty to a great extent.

The term magnesium as used herein and in the appended claims refers to the commercially available metal.

I claim:

1. A magnesium base alloy composed of magnesium and from about 0.5 to 5 per cent of antimony.
2. A magnesium base alloy composed of magnesium and from about 1 to 4 per cent of antimony.
3. A magnesium base alloy consisting of magnesium and about 1 per cent antimony.
4. A magnesium base alloy consisting of magnesium and about 4 per cent antimony.

EDWARD F. FISCHER.